

Oct. 14, 1924.

1,511,500

H. E. BROOKBY

PROCESS OF MAKING PLASTER BOARD

Filed Aug. 20, 1923



Fig. 1



Fig. 2

INVENTOR.  
HARRY E. BROOKBY  
BY *Langham Moore*  
ATTORNEYS.

## UNITED STATES PATENT OFFICE.

HARRY E. BROOKBY, OF EVANSTON, ILLINOIS.

## PROCESS OF MAKING PLASTER BOARD.

Application filed August 20, 1923. Serial No. 658,309.

*To all whom it may concern:*

Be it known that I, HARRY E. BROOKBY, a citizen of the United States, residing at Evanston, in the county of Cook and State 5 of Illinois, have invented new and useful Improvements in Processes of Making Plaster Board, of which the following is a specification.

This invention relates to improvements in 10 building materials and more particularly to a light weight wallboard or plaster board, and is an improvement of the invention set forth in my prior Patent No. 1,428,827, dated September 12, 1922.

15 Fabricated plaster board for some time has been used as a substitute for the customary wooden lath in buildings and plaster wallboard as a substitute for both wooden lath and plaster.

20 The fabricated boards of this character formed of a plaster body protected by fibrous cover sheets when used as wallboard or a substitute for both lath and plaster are usually of a larger size than the plaster 25 board or substitute for the lath alone and on account of the weight of the plaster body and increased size, usually 48 inches wide,  $\frac{3}{8}$  of an inch thick and from 6 to 10 feet in length, are both cumbersome and heavy.

30 It is an object of this invention to provide a light weight body for plaster wallboard with all the favorable characteristics and structural requirements of the present plaster wallboard but which will be easier to 35 handle in shipment and in application upon the building, wall or ceiling, and which while not detracting from the strength of the board will greatly reduce the cost of transportation.

40 With these and other objects in view, reference is had to the accompanying sheet of drawing which illustrates a preferred form of this invention, yet it is to be understood that minor detail changes may be made 45 without departing from the scope thereof.

In the drawings:

Figure 1 is a view in side elevation, with parts broken away, of a form of a machine that may be used in the fabrication of the 50 wallboard in accordance with this invention.

Figure 2 is a view in section of this improved wallboard illustrating the composition thereof.

55 The normal consistency of calcined gyp-

sum varies in water carrying capacity from 60 cubic centimeters to 90 cubic centimeters per 100 grams of gypsum depending upon the fineness, method of calcination and other factors known to the trade when calcined gypsum is produced. It has been determined that the same gypsum can be given an artificial consistency of 250 cubic centimeters, or more, of water carrying capacity to 100 grams of gypsum by agitating or 65 rapidly stirring the gypsum in such an excess of water until the mixture is in a partly "set" condition. Gypsum so treated when "set" loses considerable strength due to loss in density, is very porous when the excess 70 water evaporates and is much lighter in weight, weighing approximately one third as much per cubic centimeter as the normal mixture of gypsum and water when set. Likewise it has been determined that while 75 gypsum treated in the above manner will not bond to paper or the fibrous cover sheets for plaster wallboard, such gypsum will bond to paper coated with a gypsum and water mixture of the normal or low water 80 carrying consistency.

In producing wallboard in accordance with this invention, same character of machine as illustrated in my prior Patent 1,428,827, dated September 12, 1922, may be 85 employed which is of the usual general construction as heretofore used in the manufacture of plaster wallboard and comprises a base 1 with spaced apart supports 2 supporting rolls of paper 3 of the proper width and 90 character for the cover sheets 4 and 5 of the wallboard. An endless belt 6 passes over rollers on the base which supports the bottom cover sheet 4 between the supports 2 and the encased board after it leaves the 95 forming mechanism 7'. The forming mechanism comprises means for turning over the edges of the lower cover sheet 4 to enclose the edges of the wallboard before the feeding of the upper cover sheet 5 thereover, all 100 of which construction is well known in this art.

Conveyors 7 and 8 are provided adjacent each paper roll support 2 with a third conveyor 9 interposed between them. These 105 conveyors are all the same general construction and used in conveying a plastic mixture of calcined gypsum, sawdust and water and depositing the plastic mass upon the bottom cover sheet in the fabrication of plaster 110

wallboard, however, in this case, the outer conveyors are utilized to deposit a thin layer of calcined gypsum 10 while the intermediate conveyor deposits a plastic mass of gypsum and the desired excess of water agitated by rapidly moving stirring arms 13 upon the conveyor belt to form the light weight core 11. The three conveyors are spaced sufficient distances apart to allow sufficient 10 set of the plastic bottom layer on the under cover sheet, of the core mixture and of the plastic upper layer thereon and allow for the spreading of each, preferably by spreading rolls 12, without intermingling the ingredients before the application of the upper cover sheet. The remainder of the machine is preferably of the usual construction.

It is therefore seen that by this method a composition wallboard is formed which comprises a core 11 lighter in weight than calcined gypsum having a layer 10 on each side that bonds thereto and to the cover sheets.

The agitating or rapidly stirring the calcined gypsum in a large excess of water to 25 carry the mixture partly into "set" causes the gypsum to take up approximately three times the normal amount of water as when mixed and allowed to "set" without agitation. The agitated mixture carrying the excess water is less dense than the normal mixture and when set and the excess water evaporated, an expanded, cellular, porous body of calcined gypsum is formed which on account of its construction is not only lighter 30 but also of less structural strength than the normal set gypsum, however, as the cover sheets of wallboard impart the tensile strength to the board, a core of this form of gypsum when bonded by a layer of normal calcined gypsum to the cover sheets produces 35 a wallboard of the same tensile strength but lighter in weight than the normal gypsum wallboard.

The usual aggregates, such as sawdust, 40 may be added before or during the mixing of the gypsum with the excess of water in the same manner as in forming plaster wallboard with the normal mixture of gypsum and water.

What I claim is:

1. A plaster wallboard comprising fibrous cover sheets with layers of cementitious material bonded thereto and a core of the same material in a highly porous form bonded to said layers.

2. A plaster wallboard comprising fibrous cover sheets with layers of calcined gypsum bonded thereto and a core of light weight porous gypsum therebetween and bonded thereto.

3. A plaster wallboard comprising fibrous cover sheets with layers of normal calcined gypsum bonded thereto and a core of expanded cellular gypsum therebetween.

4. A plaster wallboard comprising a core of expanded cellular calcined gypsum with a thin layer of normal calcined gypsum on each side bonded thereto and cover sheets bonded to the gypsum layers.

5. The method of producing composition wallboard comprising the provision of a cover sheet, depositing thereon a layer of plastic cementitious material adapted to bond thereto, depositing on such layer a core of the same material adapted to produce an expanded cellular body and adapted to bond to said layer, depositing upon the core a layer of the same material as the first and laying a second cover sheet over said last layer.

6. The method of producing plaster wallboard comprising the provision of a cover sheet, depositing a layer of plastic calcined gypsum thereon, depositing on such layer a core adapted to produce a light weight porous calcined gypsum body, depositing upon the core a layer of plastic calcined gypsum and laying a cover sheet upon said last layer.

7. The method of producing plaster wallboard comprising the provision of a cover sheet, forming a thin layer of normal plastic calcined gypsum thereon, forming a core adapted to produce an expanded cellular calcined gypsum body thereon, forming a thin layer of normal plastic calcined gypsum on the core and providing a cover sheet upon the last layer.

HARRY E. BROOKBY.